

# United States Patent Office

2,991,162

Patented July 4, 1961

1

2,991,162

## MOTOR FUEL COMPOSITION

Robert E. Malec, Chicago, Ill., assignor to Standard Oil Company, Chicago, Ill., a corporation of Indiana  
No Drawing. Filed May 11, 1960, Ser. No. 28,245  
19 Claims. (Cl. 44—58)

The present invention relates to an improved motor fuel composition for spark-ignition internal combustion engines, and more particularly to such motor fuel compositions containing an additive which functions to inhibit or to reduce deposits in the induction system of spark-ignition internal combustion engines.

Rough idling and engine stalling requiring frequent carburetor adjustments and reconditioning have been problems in certain kinds of automotive engine service. These problems have been accentuated with increased traffic in congested areas and the use of multi-throat carburetors in private passenger cars. It has been determined that a primary factor in poor idling operation is an accumulation of deposits in the throttle body section of the carburetor which causes an over-rich mixture at idle and a reduction in idle speed. The accumulation of deposits in the induction system of the engine and particularly in the throttle section of the carburetor is particularly pronounced in services requiring considerable idling such as taxicab and door-to-door delivery service. In private automobile operation, this problem is particularly emphasized in the metropolitan areas where heavy city traffic is encountered with appreciable stop-and-go driving.

The critical accumulation point for these deposits is adjacent to the throttle plate, whose position controls the air-fuel ratio. As these deposits accumulate, the air flow at idle is restricted with no change in fuel flow, and a rich mixture results causing erratic idling and engine stalling. In order to compensate for the presence of these deposits, the throttle must be opened slightly by increasing the idle speed adjustment which, although allowing more air flow, automatically supplies more fuel. This requires a fuel correction by changing the idle mixture adjustment screw a compensating amount. The amount of idle adjustment required to maintain satisfactory idle performance is an indication of the rate of deposit build-up. Furthermore, deposits will often form in the idle air passageway causing restriction which allows manifold vacuum to draw more gasoline into the engine, again causing rich idle and engine stalling.

It has been established that the primary source of these deposits is the contaminants in the intake air of the engine when operating at idle. The greatest source of these intake air contaminants is engine blow-by, which accounts for approximately one-half of the deposits. Exhaust from other vehicles, dust, and other components classed as normal air pollutants contribute to the formation of deposits.

It is accordingly an object of the present invention to provide a motor fuel composition for spark-ignition internal combustion engines which will inhibit or alleviate deposits in the induction system of such engines. Another object of the invention is to provide a motor fuel composition for spark-ignition internal combustion engines which will prevent rough idling and stalling of such engines due to the accumulation of deposits in the induction system of such engines. Still another object of the invention is to provide a motor fuel composition which will remove deposits from the induction system of spark-ignition internal combustion engines. A further object of this invention is to provide an additive concentrate, which when added in small amounts to a motor fuel for spark-ignition internal combustion engines will inhibit or reduce deposits in the induction system of such engines. It is also an object of this invention to provide a method

2

of removing blow-by deposits accumulated in the induction system of spark-ignition internal combustion engines. Further, objects and advantages of the herein described invention will become apparent from the following description thereof.

In accordance with the present invention, the foregoing objects are attained by incorporating in a motor fuel for spark-ignition internal combustion engines, particularly in a hydrocarbon fuel in the gasoline distillation range, a small amount, sufficient to inhibit or reduce deposits in the induction system of such engines, from about 0.0005% to about 0.5% preferably from about 0.001% to about 0.01%, based on the hydrocarbon fuel, of a mixture consisting essentially of (1) a hydroxy-alkyl 3-(N-alkyl-amino)-propylcarbamate or hydroxyalkyl 3-(N-alkenyl-amino)-propylcarbamate and (2) an N-alkyl or N-alkenyl substituted propylene urea in the ratio of from about 1:2 to about 2:1, and preferably about 1:1 respectively.

Suitable carbamates are those having the general formula



in which R is an acyclic aliphatic radical, i.e. an alkyl or alkylene radical, having from about 8 to about 32 carbon atoms, and is preferably an alkyl group of from about 10 to about 20 carbon atoms derived from a fatty acid or mixed fatty acids, and R<sup>1</sup>, R<sup>2</sup>, R<sup>3</sup> and R<sup>4</sup> are hydrogen or an alkyl radical of from about 1 to about 4 carbon atoms. When R<sup>1</sup>, R<sup>2</sup>, R<sup>3</sup> and R<sup>4</sup> are alkyl radicals, they can be the same or different alkyl radical.

Suitable ureas are those having the general formula



wherein R is as above described, and can be the same or different alkyl or alkylene radical.

Examples of suitable carbamates are:



Suitable cyclic ureas are illustrated by the following examples:





ester carburetor is used in making the test. A vacuum port for distributor spark advance is provided in the carburetor throat area, and is normally located in the atmospheric pressure area during idling. As deposits build upon the throttle bore, it is necessary to open the throttle valve more to provide the same air flow for the same r.p.m. When this is done, the vacuum port then is partially in the manifold vacuum area. At the start of the test the vacuum on the port is about 2 to 3 inches of mercury. The failure point of the test is considered reached when this vacuum increases about 8 inches of mercury, i.e. when the port vacuum reaches 10 to 11 inches of mercury. To increase the severity of the test, all of the crankcase blow-by and some of the exhaust are admitted to the carburetor. The time required for the base fuel (control) to fail is about 20 hours, i.e. the time required for the vacuum to increase 8 inches of mercury when using the control fuel. During the test the engine is operated on a three (3) minute cycle of 2.75 minutes at 500 r.p.m. idle and 0.25 minute at 1600 r.p.m. with no load. Throttle opening and mixture adjustments are made every hour, if necessary, to maintain a 500 r.p.m. idle speed.

The improvement factor is calculated by:

$$\frac{\text{Time required for failure on fuel containing the additive}}{\text{Time required for failure on base fuel}} = \text{improvement factor}$$

The results of the test are expressed in terms of the "improvement factor" as above defined. The base motor fuel employed was a commercial premium gasoline containing the usual additives, i.e. tetraethyl lead, scavengers, antioxidant, metal deactivator, etc.

Table I

| Sample No. | Fuel                                                           | Improvement Factor         |
|------------|----------------------------------------------------------------|----------------------------|
| 1.         | Base Fuel                                                      | 1.0                        |
| 2.         | No. 1+24 p.p.m. Product Example I                              | 5.7, 4.0, 3.5<br>(av. 4.4) |
| 3.         | No. 1+24 p.p.m. Product Example II                             | 1.0                        |
| 4.         | No. 1+24 p.p.m. Product Example III                            | 2.0                        |
| 5.         | No. 1+24 p.p.m. Product Example IV                             | 3.6                        |
| 6.         | No. 1+24 p.p.m. Product Example V                              | 1.0                        |
| 7.         | No. 1+24 p.p.m. Product Example VI                             | 2.0                        |
| 8.         | No. 1+12 p.p.m. Product Example V+12 p.p.m. Product Example VI | 4.5                        |
| 9.         | No. 1+8 p.p.m. Product Example V+16 p.p.m. Product Example VI  | 3.3                        |
| 10.        | No. 1+16 p.p.m. Product Example V+8 p.p.m. Product Example VI  | 2.5                        |
| 11.        | No. 1+12 p.p.m. Product Example VII                            | 2.0                        |
| 12.        | No. 1+16 p.p.m. Product Example VII                            | 3.1, 3.0<br>(av. 3.05)     |
| 13.        | No. 1+24 p.p.m. Product Example VII                            | 3.4                        |
| 14.        | No. 1+24 p.p.m. Product Example VIII                           | 3.5                        |

In addition to the above test data, gasoline compositions of the present invention were subjected to extensive tests in laboratory engines and in the field. In the laboratory gasolines containing the carbamate-urea mixture of this invention passed the Chevrolet induction system deposit (ISD) test, the CFR L-head surface ignition test and the spark plug fouling test. Further, the defined mixture demonstrated no deleterious effects on the initial, or storage stability of the base gasoline. Gasolines containing the defined carbamate-urea mixture were field tested in a fleet of taxi-cabs over an extended period of time with periodic inspections of the induction systems, particularly the carburetors of the test cabs. In this test it was observed that the test gasolines inhibited induction system deposits as well as effectively removed existing deposits. As a result the cabs operating on the test fuels gave continuous satisfactory service extending beyond periods when normally carburetor adjustments or overhauling was to be expected.

Motor fuels containing the carbamate-urea mixture herein described can contain in addition thereto well

known antioxidants, stabilizers, anti-icing agents, anti-knock agents, scavenging agents and/or other additives which are commonly employed in motor fuels for spark-ignition internal combustion engines.

5. Percentages given herein and in the appended claims are weight percentages unless otherwise stated.

I claim:

1. A motor fuel composition comprising a major proportion of a hydrocarbon base fuel distilling within the gasoline distillation range and from about 0.0005% to about 0.5% of a mixture of (1) a carbamate selected from the group consisting of a hydroxyalkyl 3-(N-alkylamino)-propylcarbamate and a hydroxyalkyl 3-(N-alkenylamino)-propylcarbamate having the general formula



15 20 in which R is an acyclic aliphatic hydrocarbon radical having from about 8 to about 32 carbon atoms, and R<sup>1</sup>, R<sup>2</sup>, R<sup>3</sup> and R<sup>4</sup> are selected from the group consisting of hydrogen, an alkyl radical of from about 1 to about 4 carbon atoms and mixtures thereof, and (2) a substituted propylene urea having the general formula



30 35 in which R is an acyclic aliphatic hydrocarbons radical having from about 8 to about 32 carbon atoms, said carbamate and said cyclic urea being present in said mixture in the weight ratio of from about 2:1 to about 1:2.

2. A motor fuel composition as described in claim 1 wherein R is an alkyl radical of from about 8 to about 18 carbon atoms derived from mixed fatty acids, and R<sup>1</sup>, R<sup>2</sup>, R<sup>3</sup> and R<sup>4</sup> are hydrogen.

40 45 3. A motor fuel composition to spark-ignition internal combustion engines comprising a major amount of a hydrocarbon base fuel distilling within the gasoline distillation range, a tetraalkyl lead anti-knock agent and from about 0.0005% to about 0.05% of a mixture of (1) a 2-hydroxyethyl 3-(N-alkylamino)-propylcarbamate having the general formula



50 and (2) a substituted propylene urea having the general formula



55 60 65 where R is an alkyl group of from about 8 to about 32 carbon atoms, said carbamate and said urea being present in said mixture in the weight ratio of from about 2:1 to about 1:2.

6. A motor fuel composition as described in claim 3 in which R is an alkyl group of from 8 to about 18 carbon atoms derived from coconut fatty acids, and in which said carbamate and said urea are present in said mixture in the weight ratio of about 1:1.

70 75 7. A motor fuel composition as described in claim 3 in which the tetra alkyl lead anti-knock agent is tetraethyl lead.

8. A motor fuel composition as described in claim 3 in which R is an oleyl radical.

7. A motor fuel composition for spark-ignition internal combustion engines comprising a major amount of a hydrocarbon base fuel distilling within the gasoline distillation range, a tetraalkyl lead anti-knock agent and from about 0.0005% to about 0.05% of a mixture consisting of (1) a 2-hydroxypropyl 3-(N-alkylamine)-propylcarbamate having the general formula



and (2) a substituted propylene urea having the general formula



where R is an alkyl group of from about 8 to about 32 carbon atoms, said carbamate and said urea being present in said mixture in the weight ratio of from about 2:1 to about 1:2.

about 1:2.

8. A motor fuel composition as described in claim 7 in which R is an alkyl group of from 8 to about 18 carbon atoms derived from coconut fatty acids, and in which said carbamate and said urea are present in said mixture in the weight ratio of about 1:1.

9. A motor fuel composition as described in claim 7 in which the tetra alkyl lead anti-knock agent is tetraethyl lead.

10. A motor fuel composition as described in claim 7 in which R is an oleyl radical.

11. An additive for use in small amounts in hydrocarbon fuels of the gasoline boiling range adapted for use in spark-ignition internal combustion engines to maintain the induction system of such engines essentially free of deposits, said additive consisting essentially of a mixture of (1) a carbamyl selected from the group consisting of a hydroxylalkyl 3-(N-alkylamine)-propylcarbamate and a hydroxylalkyl 3-(N-alkenylamino)-propylcarbamate having the general formula



in which R is an acyclic aliphatic hydrocarbon radical having from about 8 to about 32 carbon atoms, and R<sup>1</sup>, R<sup>2</sup>, R<sup>3</sup> and R<sup>4</sup> are selected from the group consisting of hydrogen, an alkyl radical of from about 1 to about 4 carbon atoms and mixtures thereof, and (2) a substituted propylene urea having the general formula



in which R is an acyclic aliphatic hydrocarbon radical having from about 8 to about 32 carbon atoms, said carbamate and said cyclic urea being present in said mixture in the weight ratio of from about 2:1 to about 1:2.

12. An additive for use in small amounts in leaded gasoline for spark-ignition internal combustion engines to maintain the induction system of such engines essentially free of deposits, said additive consisting essentially of a mixture of (1) a 2-hydroxyethyl 3-(N-alkylamino)-propylcarbamate having the general formula

and (2) a substituted propylene urea having the general formula



10 where R is an alkyl group of from about 8 to about 32 carbon atoms, said carbamate and said urea being present in said mixture in the weight ratio of from about 2:1 to about 1:2.

13. An additive as described in claim 12 in which R is an alkyl group of from 8 to about 18 carbon atoms derived from coconut fatty acids, and in which said carbamate and said urea are present in said mixture in the weight ratio of about 1:1.

14. An additive for use in small amounts in leaded gasoline for spark-ignition internal combustion engines to maintain the induction system of such engines essentially free of deposits, said additive consisting essentially of a mixture of (1) a 2-hydroxypropyl 3-(N-alkylamino)-propylcarbamate having the general formula



and (2) a substituted propylene urea having the general formula



15. An additive as described in claim 14 in which R is an alkyl group of from 8 to about 18 carbon atoms derived from coconut fatty acids, and in which said carbamate and said urea are present in said mixture in the weight ratio of about 1:1.

16. The method of preparing an additive for use in small amounts in hydrocarbon fuels of the gasoline boiling range adapted for use in spark-ignition internal combustion engines to maintain the induction system of such engines essentially free of deposits, which method comprises reacting molar proportions of a diamine having the general formula  $RNH(CH_2)_3NH_2$  and an alkylene carbonate having the general formula



at a temperature of from about 50° C. to about 250° C. for a time sufficient to give a reaction product consisting essentially of a mixture of a carbamate having the general formula



and a cyclic urea having the general formula



in which R is an acyclic aliphatic hydrocarbon radical having from about 8 to about 32 carbon atoms, and  $R^1$ ,

R<sup>2</sup>, R<sup>3</sup> and R<sup>4</sup> are selected from the group consisting of hydrogen, an alkyl radical of from about 1 to about 4 carbon atoms and mixtures thereof, said carbamate and said urea being present in said mixture in the weight ratio of from about 1:2 to about 2:1.

17. The method of claim 16 wherein R is an alkyl radical of about 8 to about 18 carbon atoms derived from mixed coconut fatty acids, R<sup>1</sup>, R<sup>2</sup>, R<sup>3</sup> and R<sup>4</sup> are hydrogen and wherein said carbamate and said urea are present in said mixture the weight ratio of about 1:1.

18. The method of claim 16 in which the alkylene carbonate is ethylene carbonate.

19. The method of claim 16 in which the alkylene carbonate is propylene carbonate.

References Cited in the file of this patent

UNITED STATES PATENTS

2,922,707 Lindstrom et al. ----- Jan. 26, 1960  
10 2,961,308 Andress ----- Nov. 22, 1960

UNITED STATES PATENT OFFICE  
CERTIFICATION OF CORRECTION

Patent No. 2,991,162

July 4, 1961

Robert E. Malec

It is hereby certified that error appears in the above numbered patent requiring correction and that the said Letters Patent should read as corrected below.

Column 6, line 34, for "hydrocarbons" read -- hydrocarbon --; column 7, lines 6 and 41, for "3-(N-alkylamine)-", each occurrence, read -- 3-(N-alkylamino)- --; column 8, line 36, after the formula, the following should be inserted:

where R is an alkyl group of from about 8 to about 32 carbon atoms, said carbamate and said urea being present in said mixture in the weight ratio of from about 2:1 to about 1:2.

Signed and sealed this 17th day of October 1961.

(SEAL)

Attest:

ERNEST W. SWIDER  
Attesting Officer

DAVID L. LADD  
Commissioner of Patents